# EUROPEAN PATENT SPECIFICATION

(11) **EP 4 369 970 B1**
(45) Date of publication and mention of the grant of the patent: **11.02.2026**
(21) Application number: 22826108.7
(22) Date of filing: 01.12.2022
(51) Int. Cl.: A41D 19/015, A41D 19/00

(54) **ARC FLASH PROTECTION GLOVE**
HANDSCHUH ZUM SCHUTZ VOR LICHTBÖGEN UND WÄRME
GANT DE PROTECTION CONTRE LES ÉCLAIRS D'ARC ET LA CHALEUR

(30) Priority: 01.12.2021 EP 21211844
(43) Date of publication of application: 22.05.2024
(73) Proprietor: Y. Berger & Co. AB, 438 91 Landvetter (SE)
(72) Inventor: BERGER, Markus, 1274 Gothenburg (SE)
(74) Representative: KIPA AB
(86) International application number: PCT/EP2022/084111
(87) International publication number: WO 2023/099685

(56) References cited:
- BE-A1- 1 027 761
- FR-A1- 2 981 248
- US-A1- 2015 135 403
- US-A1- 2016 120 242
- US-B2- 8 074 436

## Description

### Technical field

The present invention relates to an arc flash protection glove, a heat protection glove and a method for manufacturing said gloves.

### Background

A major hazard when working with electrical equipment is arc flashes. An arc flash occurs when an electrical connection is established through air, resulting in dispersion of energy in the form of electromagnetic radiation and heat. The amount of energy generated naturally varies with voltage levels of the electrical system in question, but normally falls within the interval of 0 to 600 Cal/cm². However, it is important to note that an arc flash releasing energy of only 2 Cal/cm² may cause second-degree burns to unprotected skin.

One way of mitigating the risk of serious injury is the use of protective gloves. There exist a variety of solutions on the market, among which US2014237701 may be mentioned. However, a common problem with existing solutions is that, although they may be fire-resistant to a certain degree, they do not provide adequate protection against arc flashes. More importantly, even if a solution provides good protection, the drawback is often loss of flexibility, wearability and mobility.

Thus, there is a need for gloves with increased arc flash protection while flexibility, wearability and mobility are retained or improved.

US 2016/0120242 A1 discloses a glove, including a fabric liner having a thumb, an index finger, a middle finger, a ring finger, a pinkie finger, a palm area, an upper knuckle area, a back of a hand area, and optionally a cuff; at least one two-dimensional injection molded component disposed on at least one planar region of the fabric liner.

FR 2 981 248 A1 discloses a thermal protection accessory and manufacturing method of a thermal protection glove for handling hot parts, possibly oily or greasy, with great dexterity and strong thermal insulation. According to the invention, this thermal protection accessory comprises a textile layer comprising a first surface and a second surface, a coating covering at least part of the first surface of the textile layer, and pins distributed on the surface of at least one area of the coating. BE 1 027 761 A1 discloses a fire resistant glove suitable for security personnel such as police or fire brigade, wherein this glove is composed of a laminated textile system, where this textile system comprises an outer textile system and an inner textile system, which outer textile system includes multiple strips of different materials and where the inner textile system is composed of three layers, a waterproof membrane layer, a para-aramid layer and a meta-aramid layer, and where the fire resistant glove complies with the safety requirements of Regulation (EU) 2016/425.

US 8,074,436 B2 discloses a flexible cut resistant hydrocarbon flash fire resistant latex glove article that has a flame-resistant cut resistant liner and a flame-resistant oil resistant polychloroprene polymeric latex coating. The knitted cut resistant fire-resistant liner has is made from a composite yarn having a fiberglass core and optionally including a steel fibre. The core has a cushioning core sheath formed by ringspinning of microdenier staple cut resistant fibres of, for example, para-aramid. Staple modacrylic fibres can be included with the staple para-aramid fibres. Two wraps of continuous yarns of polyester, para-aramid, or both at a wrap density such that the wraps do not cover the core sheath in its entirety. In the absence of steel fibre, the cut resistant hydrocarbon flash fire resistant glove exhibits good electrical insulation characteristics even with sweat generated from hand preventing short circuit of electrical circuits. The glove is flexible due to the low denier of the composite yarn and is highly breathable especially when only the palm and fingers are coated with polychloroprene polymer.

### Summary

An object of the present invention is therefore to overcome the above problems, and to provide a solution that at least to some extent improve upon the prior art. This, and other objects, which will become apparent in the following, is accomplished by the arc flash and heat protection glove defined in the accompanying claims.

According to another aspect of the invention, a method for manufacturing an arc flash protection and fire-resistant glove is provided, the method is according to claim 12.

### Brief description of the drawings

These and other variants of the present invention will now be described in more detail, with reference to the appended drawings showing exemplary embodiments of the present invention, wherein:
Fig. 1 is a schematic perspective view of a palm side and a backside of a glove liner.
Fig 2 is a schematic perspective view of a palm side and a backside glove according to the first aspect, second aspect or third aspect of the present invention comprising a continuous backside coating.
Fig. 3 is a schematic perspective view of a glove according to the first aspect, second aspect or third aspect of the present invention comprising a discontinuous backside coating comprising a dot pattern.

### Detailed description of the drawings

In Fig. 1, a fire-resistant glove liner 2 is depicted. The fire-resistant glove liner 2 may be formed of a fire-resistant material selected from the group consisting of: para-aramid, meta-aramid, modacrylic, cotton, wool, polyamide and polyester, or any combination thereof. The fire-resistant glove liner 2 consists of a palm side 3 and a backside 4. The palm side 3 comprises palm side finger portions 3A, a palm side center portion 3B and a palm side cuff portion 3C. The backside 4 comprises backside finger portions 4A, a backside center portion 4B and a backside cuff portion 4C. This glove liner comprises five finger portions. In Fig. 1, the respective portions are delimited with lines.

In Fig. 2, an arc flash and heat protection glove 100 is shown. The glove 100 is shown in both a palm side view (left hand side) and backside view (right hand side). The glove 100 comprises a fire-resistant glove liner 2, as seen in Fig. 1. The glove liner is provided with a fire-resistant coating 5 comprising a fire-resistant material. A fire-resistant material may comprise polymers selected from the group consisting of silicon, polyvinylchloride and chloroprene, or a mixture thereof. For example, the fire-resistant material may comprise 10 - 90 wt% chloroprene, or 20 - 80 wt% chloroprene, or 30 - 70 wt% chloroprene, or 40 - 60 wt% chloroprene.

A fire-resistant coating 5 may further comprise an additive selected from the group consisting of: pigments, fillers, softeners, surface active agents, accelerators, crosslinkers and vulcanizers, or mixtures thereof. The additive and the fire-resistant material may be provided in a fire-resistant coating composition, optionally together with a solvent.

According to one example the fire-resistant composition comprises Chloropren and 5 pph (part per hundred) of ZnO. According to a alternative example the fire-resistant composition comprises PVC, which is thermally treated together with 60 pph of a softener such as DINCH (1,2-Cyclohexane dicarboxylic acid diisononyl ester).

The fire-resistant coating 5 comprises a palm side coating portion 5A. The palm side coating portion 5A is arranged on the palm side 3 of the glove liner 2. Here, the palm side coating portion 5A covers at least 90% of the palm side finger portions 3A and at least 90% of the palm side center portion 4B. Alternatively, the palm side coating portion 5A may cover at least 95% of the palm side finger portions 3A and at least 95% of the palm side center portion 4B. Alternatively, the palm side coating portion 5A may fully cover the palm side 3 finger portions 3A and the palm side center portion 4B.

The fire-resistant coating 5 further comprises a backside coating portion 5B. The backside coating portion 5B is arranged on the backside center portion 4B. The backside coating portion 5B is arranged on at least 4 cm² of the backside center portion 4B. As is seen in Fig. 2, the backside 4 is provided with at least at least 4 cm² of a backside coating portion 5B, as indicated by the dashed square on the backside coating portion 5B. For reference, a corresponding square is shown on the palm side. Alternatively, the backside coating portion 5B may have an area of at least 5 cm², or at least 6 cm², or at least 7 cm², or at least 8 cm². The backside coating portion 5B is deposited as at least one layer that is thinner and/or has a different material composition than the palm side coating portion 5A. In Fig. 1, the backside coating portion 5B is arranged as a continuous layer of an area of at least 4 cm² on the backside center portion 4B. Here, the continuous layer of the backside coating portion 5B is arranged on the entire area of the backside center portion 4B. Furthermore, the backaside coating portion 5B is arranged on at least 80% of the backside finger portions 4A.

The glove 100 was e.g. manufactured by providing a first coating to the glove liner (not shown), subsequently providing a second coating, e.g. by a palm dip such that the palm side finger portions 3A and the palm side center portion 3B is fully covered by the second coating. Furthermore, the second coating was, e.g. during the palm dip, provided to a portion of the backside finger portions 4A. The glove 100 was e.g. subsequently provided with a third coating on the backside center portion, fully covering the backside center portion, and on a portion of the backside finger portions 4A.

The backside coating portion 5B is fully or partly composed of a different fire-resistant material compared to the palm side coating portion 5A. Hereby, the backside coating portion 5B and the palm side coating portion 5A may have substantially different properties. For example, the palm side coating portion 5A may have a higher fire-resistance than the backside coating portion 5B, or vice versa. As another example, the backside coating portion 5B may be composed of a lighter fire-resistant material compared to the palm side coating portion 5A. The palm side coating portion 5A may e.g. comprise a first layer of a first material, and the backside coating portion 5B may comprise a first layer of the first material, wherein the palm side coating portion 5A or the backside coating portion 5B comprise a second layer of a second material.

The average coating weight of the backside coating portion 5B is within the range of 5-80% of the average coating weight of the palm side coating portion 5A. The darker coating present i.a. on the palm side coating portion may have a total coating weight within the range of 5-20 g/glove of size 10. The brighter coating present i.a. on the backside coating portion may have a total coating weight in the range of 1-8 g/glove of size 10. This is scaleable to gloves of other sizes as explained above.

Fig. 3 depicts an arc flash and heat protection glove 200 where the backside coating portion 5B is arranged as a discontinuous layer. The glove 200 is shown in both a palm side view (left hand side) and backside view (right hand side). The discontinuous layer is arranged on an area of at least 4 cm² on the backside center portion 4B. Here, the discontinuous backside coating portion 5B comprises a dot pattern. Here, the dots 6 comprised in the dot pattern are depicted as being distributed in a uniform manner over the backside center portion 4B, such that any dot 6 has the same separation distance to any closest neighbor of the dot 6. The dot pattern may e.g. comprise dots 6 that are 1-3 mm in diameter, with a separation distance of 1-3 mm. Alternatively, the dots 6 comprised in the dot pattern may be nonuniform in size. Furthermore, the dots 6 comprised in the dot pattern may be nonuniform in separation distance, such that some dots 6 are arranged closer to any closest neighbor as compared to other dots 6. For example, the dot pattern may comprise dots that are alternating in size, such that half the dots are larger than the other half. For example, half the dots may be 3-6 mm in diameter while the other half may be 1-3 mm in diameter.

The gloves 100 and 200 in Fig. 2 and 3 may be manufactured by the same method. A method for manufacturing an arc flash protection or fire-resistant glove is provided according to the fourth aspect of the present invention. First, a fire-resistant glove liner 2 is provided. The glove liner 2 consists of a palm side 3 and a backside 4, which backside 4 comprises backside finger portions 4A, a backside center portion 4B and a backside cuff portion 4C.

A fire-resistant coating 5 is subsequently provided to the glove liner 2. The fire-resistant coating 5 is applied by providing a backside coating portion 5B having an area of at least 4 cm² on the backside center portion 4B, and providing a palm side coating portion 5A on the palm side 3, wherein the palm side coating portion 5A covers at least 90% of the palm side 3. The backside coating portion 5B may be arranged in a continuous layer, as is shown in Fig. 2 and discussed in relation to said figure above, or in a discontinuous layer, as is shown in Fig. 3 and discussed in relation to said figure above.

An average coating weight, after the palm side coating portion 5A and the backside coating portion 5B have been applied, of the backside coating portion 5B is within the range of 5-80% of an average coating weight of the palm side coating portion 5A. An average coating weight of said backside coating portion is alternatively within the range of 10-70%, or 15-60%, or 20-55%, or 25-50% of an average coating weight of said palm side coating portion. An estimation of the coating weight may be made: by cutting a 4 cm² piece of the backside center portion 4B and a 4 cm² piece of e.g. the palm side center portion, weigh the separate pieces, divide the respective weights with 4 cm² each and calculate the ratio therebetween. A more thorough way of measuring the coating weight is subtracting the dry weight of the glove liner 2 before the step of providing fire-resistant coating 5 from the dry weight of the coated glove liner 2.

According to the invention, the method comprises providing at least one fire-resistant coating composition for the backside center portion 4B, and providing at least one fire-resistant coating composition for said palm side 3. The step of providing a backside coating on said backside center portion 4B may thus further comprise providing at least one layer of the at least one fire-resistant coating composition for the backside center portion 4B to the backside center portion 4B. Correspondingly, the step of providing a palm side coating 5A on the palm side 3 further comprises providing at least one layer of the at least one fire-resistant coating composition for the palm side 3 to the palm side 3. The backside center portion 4B and the palm side 3 may be provided with a different number of layers.

Furthermore, any layer applied to the palm side 3 may be thicker or thinner than any layer applied to the backside center portion 4B, or vice versa.

The step of providing a backside coating 5B may further comprise providing a plurality of layers of the fire-resistant material composition on top of each other. Furthermore, the step of providing a palm side coating portion 5A comprises providing a plurality of layers of the palm coating composition on top of each other. A predetermined number of the plurality of layers of the backside coating 5B and a predetermined number of the plurality of layers of the palm side coating 5A may be provided simultaneously. Optionally, the total number of layers of the palm side coating 5A provided to the palm side 3 is larger than total number of layers of the backside coating 5B provided to the backside center portion 4B.

Furthermore, the fire-resistant coating composition for the palm side 3 and the fire-resistant coating composition for the backside 4 is different. As such, the compositions may comprise different fire-resistant materials, and/or different additives, leading the coating compositions to provide different properties to the sides to which they are applied. For example, the backside center portion 4B may be provided with a first layer of a first composition, and the palm side 3 may be provided with a first layer of the first composition, whereafter the palm side coating portion 5A or the backside coating portion 5B may be provided with a layer of a second composition.

Providing the backside coating 5B and/or said palm side coating 5A may be performed by a method comprising dipping, spraying, brushing or screen-printing, or a combination thereof. For example, the glove liner 2 may first be subjected to dipping. The glove liner 2 may e.g. be subjected to three-quarter dipping. Alternatively, the glove liner 2 may be subjected to a palm dip, knuckle dip, finger dip, half-dip, or full dip, or a combination thereof. For example, the glove liner 2 may be subjected to dipping such that a palm side coating portion 5A is applied. Subsequently, the glove liner 2 may be subjected to spraying, brushing or screen-printing such that a backside coating portion 5B is applied.

The step of providing the backside coating may comprise providing a discontinuous coating. The step of providing a discontinuous coating may be performed by means of spraying or screen-printing the at least one fire-resistant coating composition for the backside center portion 4B on the backside center portion 4B. The discontinuous coating may be provided by use of a template through which the coating material passes before being deposited on the backside center portion 4B.

In some embodiments, the glove liner 2 may be mounted on a mould. By mounting the glove liner 2 on a mould, it is for some coating methods easier to coat the liner 2. A flat mould may be used. The flat mould may have a non rectangular transection measured across the finger. The flat mould may e.g. be a flat mould as disclosed in the registered design RCD-007571237. Alternatively, the glove liner 2 may be mounted on a hand shaped mould, such as an aluminum mould.

The glove liner 2 may optionally be washed in water. The glove liner 2 may be washed in water on the mould, alternatively off the mould before being mounted on the mould. During washing, the glove liner is dipped into water, ethanol or methanol with dissolved electrolytes such as CaCl2, Ca(NO3)2 or similar.

The coating composition or coating compositions may, after having been applied to the glove liner 2, be subjected to drying of the coating composition to yield a fire-resistant coating material. The step of drying may comprise application of heat through convection, radiation or conduction, or a combination thereof. The step of drying may be performed with in an oven.

The coating composition may be subjected to two steps of drying. For example, the coating composition may be pre-dried after it has been provided to the glove liner 2. After pre-drying, the composition is washed by dipping the coated glove liner into water, ethanol or methanol with dissolved electrolytes such as CaCl2, Ca(NO3)2. After washing, the coated glove liner 2 may be subjected to final drying.

The coating glove liner 2 may also be subjected to salt texturing or a second dip in a coagulant in order to stabilize the coating.

A step of vulcanization of the coating composition on the glove liner 2 may optionally be employed. The vulcanization temperature may be within the range of 80-140 °C, or 85-135 °C , or 90 - 130 °C.

## Claims

1. An arc flash and heat protection glove (100, 200) comprising a fire-resistant glove liner (2), which glove liner (2) consists of a palm side (3) and a backside (4), which palm side (3) comprises palm side finger portions (3A), a palm side center portion (3B) and a palm side cuff portion (3C), which backside (4) comprises backside finger portions (4A), a backside center portion (4B) and a backside cuff portion (4C), which glove liner (2) is provided with a fire-resistant coating comprising a fire-resistant material, said fire-resistant coating comprises:
a backside coating portion (5B) having an area of at least 4 cm² and being arranged on the backside center portion (4B), and
a palm side coating portion (5A) arranged on the palm side (3) of said glove liner (2),
wherein said palm side coating portion (5A) covers at least 90% of said palm side finger portions (3A) and at least 90% of said palm side center portion (3B),
wherein an average coating weight of said backside coating portion (5B) is within the range of 5-80% of an average coating weight of said palm side coating portion (5A) **characterized in that**
said backside coating portion (5B) is fully or partly composed of a different fire-resistant material compared to the palm side coating portion (5A).

2. The glove according to claim 1, wherein said back side coating portion (5B) is arranged as a continuous layer.

3. The glove according to claim 1, wherein said back side coating portion (5B) is arranged as a discontinuous layer.

4. The glove according to claim 3, wherein said discontinuous layer comprises a dot pattern.

5. The glove according to claim 4, wherein dots (6) comprised in said dot pattern are being distributed in a uniform manner over the backside center portion (4B).

6. The glove according to any one of claims 1 to 5, comprising a first coating arranged on at least said palm side (5A) coating portion, which first coating has a total coating weight within the range of 5-20 g/glove of size 10, size given according to the standard EN 21420; and comprising a second coating arranged on at least said backside (5B) coating portion, which second coating has a total coating weight within the range of 1-8 g/glove of size 10.

7. The glove according to any one of claims 1 to 6, comprising a first coating arranged on at least said palm side (5A) coating portion, which first coating has a total coating weight within the range of 3.3-25 g; and comprising a second coating arranged on at least said backside (5B) coating portion, which second coating has a total coating weight within the range of 0.66 - 10 g.

8. The glove according to any one of claims 1 to 7, wherein the fire-resistant material comprises polymers selected from the group consisting of silicon, polyvinylchloride and chloroprene, or a mixture thereof.

9. The glove according to claim 8, wherein the fire-resistant material comprises 10 - 90 wt% chloroprene, or 20 - 80 wt% chloroprene, or 30 - 70 wt% chloroprene, or 40 - 60 wt% chloroprene.

10. The glove according to any one of claims 1 to 9, wherein the fire-resistant coating further comprises an additive selected from the group consisting of: pigments, fillers, softeners, surface active agents, accelerators, crosslinkers and vulcanizers, or mixtures thereof.

11. The glove according to any one of claims 1 to 10, wherein the glove liner (2) is formed of a fire-resistant material selected from the group consisting of: para-aramid, meta-aramid, modacrylic, cotton, wool, polyamide and polyester.

12. A method for manufacturing an arc flash protection and fire-resistant glove (100, 200) comprising the steps of:
- providing a fire-resistant glove liner (2), which glove liner (2) consists of a palm side (3) and a backside (4), which palm side (3) comprises palm side finger portions (3A), a palm side center portion (3B) and a palm side cuff portion (3C), which backside (4) comprises backside finger portions (4A), a backside center portion (4B) and a backside cuff portion (4C);
- providing a fire-resistant coating to said glove liner (2) by:
providing a backside coating portion (5B) having an area of at least 4 cm² on said backside center portion (4B); and
providing a palm side coating portion (5A) on said palm side (3), wherein said palm side coating portion (5A) covers at least 90% of said palm side finger portions (3A) and at least 90% of said palm side center portion (3B);
wherein an average coating weight of said backside coating portion (5B) is within the range of 5-80% of an average coating weight of said palm side coating portion (5A); and
wherein the backside coating portion (5B) is fully or partly composed of a different fire-resistant material compared to the palm side coating portion (5A).

13. The method according to claim 12, further comprising the steps of:
- providing at least one fire-resistant coating composition for said backside center portion (4B),
- providing at least one fire-resistant coating composition for said palm side (3), and
- wherein said step of providing a backside coating on said backside center portion (4B) further comprises providing at least one layer of said at least one fire-resistant coating composition for said backside center portion (4B) to said backside center portion (4B),
- wherein said step of providing a palm side coating on said palm side (3) further comprises providing at least one layer of said at least one fire-resistant coating composition for said palm side (3) to said palm side (3),
and wherein said fire-resistant coating composition for said palm side (3) and said fire-resistant coating composition for said backside (4) different.

14. The method according to claim 13, wherein said step of providing a backside coating portion (5B) further comprises providing a plurality of layers of said fire-resistant material composition on top of each other, and said step of providing a palm side coating portion (5A) comprises providing a plurality of layers of said palm coating composition (5A) on top of each other, wherein
a predetermined number of said plurality of layers of said back side coating portion (5B) and a predetermined number of said plurality of layers of said palm side coating portion (5A) are provided simultaneously, e.g. by means of dipping or spray coating; and optionally the total number of layers of said palm side coating portion (5A) provided to said palm side (3) is larger than total number of layers of said backside coating portion (5B) provided to said backside center portion (4B).

15. The method according to claim 12 to 14, wherein the step of providing said backside coating portion (5B) and/or said palm side coating portion (4B) is performed by a method comprising dipping, spraying, brushing or screen-printing, or a combination thereof.

16. The method according to claim 15 wherein the step of providing said backside coating portion (5B) comprises providing a discontinuous coating by means of spraying or screen-printing said at least one fire-resistant coating composition for said backside center portion (4B).

## Patentansprüche

1. Ein Handschuh zum Schutz vor Lichtbögen und Feuer (100, 200) mit einem feuerfesten Handschuhfutter (2), wobei das Handschuhfutter (2) aus einer Handflächenseite (3) und einer Rückseite (4) besteht, wobei die Handflächenseite (3) handflächenseitige Fingerabschnitte (3A), einen handflächenseitigen Mittelabschnitt (3B) und einen handflächenseitigen Stulpenabschnitt (3C) umfasst, die Rückseite (4) rückseitige Fingerabschnitte (4A), einen rückseitigen Mittelabschnitt (4B) und einen rückseitigen Stulpenabschnitt (4C) umfasst und das Handschuhfutter (2) mit einer feuerfesten Beschichtung versehen ist, die ein feuerfestes Material umfasst, wobei besagte feuerfeste Beschichtung Folgendes umfasst:
einen rückseitigen Beschichtungsabschnitt (5B) mit einer Fläche von mindestens 4 cm², der auf dem rückseitigen Mittelabschnitt (4B) angeordnet ist, und
einen handflächenseitigen Beschichtungsabschnitt (5A), der auf der Handflächenseite (3) besagten Handschuhfutters (2) angeordnet ist, wobei besagter handflächenseitiger Beschichtungsabschnitt (5A) mindestens 90 % besagter handflächenseitiger Fingerabschnitte (3A) und mindestens 90 % besagten handflächenseitigen Mittelabschnitts (3B) bedeckt,
wobei ein durchschnittliches Beschichtungsgewicht des rückseitigen Beschichtungsabschnitts (5B) im Bereich von 5 bis 80 % eines durchschnittlichen Beschichtungsgewichts des handflächenseitigen Beschichtungsabschnitts (5A) liegt, **dadurch gekennzeichnet, dass**
besagter rückseitiger Beschichtungsabschnitt (5B) vollständig oder teilweise aus einem anderen feuerfesten Material als der handflächenseitige Beschichtungsabschnitt (5A) besteht.

2. Der Handschuh gemäß Anspruch 1, wobei besagter rückseitiger Beschichtungsabschnitt (5B) als durchgehende Schicht angeordnet ist.

3. Der Handschuh gemäß Anspruch 1, wobei besagter rückseitiger Beschichtungsabschnitt (5B) als unterbrochene Schicht angeordnet ist.

4. Der Handschuh gemäß Anspruch 3, wobei besagte diskontinuierliche Schicht ein Punktemuster umfasst.

5. Der Handschuh gemäß Anspruch 4, wobei die in besagtem Punktemuster enthaltenen Punkte (6) gleichmäßig über den rückseitigen Mittelabschnitt (4B) verteilt sind.

6. Der Handschuh gemäß einem der Ansprüche 1 bis 5, umfassend eine erste Beschichtung, die mindestens auf besagtem handflächenseitigen Beschichtungsabschnitt (5A) angeordnet ist, wobei die erste Beschichtung ein Gesamtbeschichtungsgewicht im Bereich von 5 bis 20 g/Handschuh der Größe 10 gemäß der Norm EN 21420 aufweist; und eine zweite Beschichtung, die auf mindestens besagtem rückseitigen Beschichtungsabschnitt (5B) angeordnet ist, wobei die zweite Beschichtung ein Gesamtbeschichtungsgewicht im Bereich von 1 bis 8 g/Handschuh der Größe 10 aufweist.

7. Der Handschuh gemäß einem der Ansprüche 1 bis 6, umfassend eine erste Beschichtung, die mindestens auf besagtem handflächenseitigen Beschichtungsabschnitt (5A) angeordnet ist, wobei die erste Beschichtung ein Gesamtbeschichtungsgewicht im Bereich von 3,3 bis 25 g aufweist; und umfassend eine zweite Beschichtung, die mindestens auf besagtem rückseitigen Beschichtungsabschnitt (5B) angeordnet ist, wobei die zweite Beschichtung ein Gesamtbeschichtungsgewicht im Bereich von 0,66 bis 10 g aufweist.

8. Der Handschuh gemäß einem der Ansprüche 1 bis 7, wobei das feuerbeständige Material Polymere umfasst, die aus der Gruppe ausgewählt sind, die aus Silikon, Polyvinylchlorid und Chloropren oder einer Mischung davon besteht.

9. Der Handschuh gemäß Anspruch 8, wobei das feuerfeste Material 10 bis 90 Gewichtsprozent Chloropren oder 20 bis 80 Gewichtsprozent Chloropren oder 30 bis 70 Gewichtsprozent Chloropren oder 40 bis 60 Gewichtsprozent Chloropren umfasst.

10. Der Handschuh gemäß einem der Ansprüche 1 bis 9, wobei die feuerfeste Beschichtung ferner ein Additiv umfasst, das aus der Gruppe ausgewählt ist, die aus Pigmenten, Füllstoffen, Weichmachern, oberflächenaktiven Mitteln, Beschleunigern, Vernetzern und Vulkanisationsmitteln oder Mischungen davon besteht.

11. Der Handschuh gemäß einem der Ansprüche 1 bis 10, wobei das Handschuhfutter (2) aus einem feuerfesten Material gebildet wird, das aus der Gruppe ausgewählt ist, die aus Para-Aramid, Meta-Aramid, Modacryl, Baumwolle, Wolle, Polyamid und Polyester besteht.

12. Ein Verfahren zur Herstellung eines Handschuhs zum Schutz vor Lichtbögen und Feuer (100, 200) mit den folgenden Schritten:
Bereitstellen eines feuerfesten Handschuhfutters (2), wobei das Handschuhfutter (2) aus einer Handflächenseite (3) und einer Rückseite (4) besteht, wobei die Handflächenseite (3) handflächenseitige Fingerabschnitte (3A), einen handflächenseitigen Mittelabschnitt (3B) und einen handflächenseitigen Stulpenabschnitt (3C) umfasst und die Rückseite (4) rückseitige Fingerabschnitte (4A), einen rückseitigen Mittelabschnitt (4B) und einen rückseitigen Stulpenabschnitt (4C) umfasst;
Versehen besagten Handschuhfutters (2) mit einer feuerfesten Beschichtung durch:
Bereitstellen eines rückseitigen Beschichtungsabschnitts (5B) mit einer Fläche von mindestens 4 cm² auf besagtem rückseitigen Mittelabschnitt (4B); und
Bereitstellen eines handflächenseitigen Beschichtungsabschnitts (5A) auf besagter Handflächenseite (3), wobei besagter handflächenseitiger Beschichtungsabschnitt (5A) mindestens 90 % besagter handflächenseitigen Fingerabschnitte (3A) und mindestens 90 % besagten handflächenseitigen Mittelabschnitts (3B) bedeckt;
wobei ein durchschnittliches Beschichtungsgewicht besagten rückseitigen Beschichtungsabschnitts (5B) im Bereich von 5 bis 80 % eines durchschnittlichen Beschichtungsgewichts besagten handflächenseitigen Beschichtungsabschnitts (5A) liegt; und
wobei der rückseitige Beschichtungsabschnitt (5B) vollständig oder teilweise aus einem anderen feuerfesten Material besteht als der handflächenseitige Beschichtungsabschnitt (5A).

13. Das Verfahren gemäß Anspruch 12, das ferner die folgenden Schritte umfasst:
- Bereitstellen mindestens einer feuerfesten Beschichtungszusammensetzung für besagten rückseitigen Mittelabschnitt (4B),
- Bereitstellen mindestens einer feuerfesten Beschichtungszusammensetzung für besagte Handflächenseite (3) und
- wobei besagter Schritt des Bereitstellens einer rückseitigen Beschichtung für besagten rückseitigen Mittelabschnitt (4B) weiterhin das Bereitstellen mindestens einer Schicht der mindestens einen feuerfesten Beschichtungszusammensetzung für den rückseitigen Mittelabschnitt (4B) auf dem rückseitigen Mittelabschnitt (4B) umfasst,
- wobei besagter Schritt des Bereitstellens einer Beschichtung für die Handflächenseite (3) ferner das Bereitstellen mindestens einer Schicht der mindestens einen feuerfesten Beschichtungszusammensetzung für die Handflächenseite (3) für die Handflächenseite (3) umfasst,
- und wobei besagte feuerbeständige Beschichtungszusammensetzung für die Handflächenseite (3) und die feuerbeständige Beschichtungszusammensetzung für die Rückseite (4) unterschiedlich sind.

14. Das Verfahren gemäß Anspruch 13, wobei besagter Schritt des Bereitstellens eines rückseitigen Beschichtungsabschnitts (5B) ferner die Bereitstellung einer Vielzahl von Schichten der besagten feuerfesten Materialzusammensetzung übereinander umfasst, und besagter Schritt des Bereitstellens eines handflächenseitigen Beschichtungsabschnitts (5A) das Bereitstellen einer Vielzahl von Schichten des besagten handflächenseitigen Beschichtungsabschnitts (5A) übereinander umfasst, wobei
eine vorbestimmte Anzahl besagter mehrerer Schichten des besagten rückseitigen Beschichtungsabschnitts (5B) und eine vorbestimmte Anzahl der besagten mehreren Schichten des besagten handflächenseitigen Beschichtungsabschnitts (5A) gleichzeitig aufgebracht werden, z. B. durch Eintauchen oder Sprühbeschichtung; und optional die Gesamtzahl der Schichten des besagten handflächenseitigen Beschichtungsabschnitts (5A), die auf besagte Handflächenseite (3) aufgebracht werden, größer ist als die Gesamtzahl der Schichten des besagten rückseitigen Beschichtungsabschnitts (5B), die auf besagten rückseitigen Mittelabschnitt (4B) aufgebracht werden.

15. Das Verfahren gemäß Anspruch 12 bis 14, wobei der Schritt des Bereitstellens des besagten rückseitigen Beschichtungsabschnitts (5B) und/oder des besagten handflächenseitigen Beschichtungsabschnitts (4B) durch ein Verfahren erfolgt, das Eintauchen, Sprühen, Streichen oder Siebdrucken oder eine Kombination davon umfasst.

16. Das Verfahren gemäß Anspruch 15, wobei der Schritt des Bereitstellens des besagten rückseitigen Beschichtungsabschnitts (5B) das Aufbringen einer diskontinuierlichen Beschichtung durch Sprühen oder Siebdrucken der mindestens einen feuerfesten Beschichtungszusammensetzung für den besagten rückseitigen Mittelabschnitt (4B) umfasst.

## Revendications

1. Gant de protection contre les éclairs d'arc et la chaleur (100, 200) comprenant une doublure de gant résistant au feu (2), laquelle doublure de gant (2) se compose d'un côté de paume (3) et d'un côté de dos (4), lequel côté de paume (3) comprend des parties pour doigts de côté de paume (3A), une partie centrale de côté de paume (3B) et une partie pour poignet de côté de paume (3C), lequel côté de dos (4) comprend des parties pour doigts de côté de dos (4A), une partie centrale de côté de dos (4B) et une partie pour poignet de côté de dos (4C), laquelle doublure de gant (2) est dotée d'un revêtement résistant au feu comprenant un matériau résistant au feu, ledit revêtement résistant au feu comprend :
une partie de revêtement de côté de dos (5B) présentant une surface d'au moins 4 cm² et étant agencée sur la partie centrale de côté de dos (4B), et
une partie de revêtement de côté de paume (5A) agencée sur le côté de paume (3) de ladite doublure de gant (2), où ladite partie de revêtement de côté de paume (5A) couvre au moins 90 % desdites parties pour doigts de côté de paume (3A) et au moins 90 % de ladite partie centrale de côté de paume (3B),
où une masse de revêtement moyenne de ladite partie de revêtement de côté de dos (5B) se situe dans la plage allant de 5 à 80 % d'une masse de revêtement moyenne de ladite partie de revêtement de côté de paume (5A) **caractérisé en ce que**
ladite partie de revêtement de côté de dos (5B) est totalement ou partiellement composée d'un matériau résistant au feu différent par rapport à la partie de revêtement de côté de paume (5A).

2. Gant selon la revendication 1, dans lequel ladite partie de revêtement de côté de dos (5B) est agencée sous la forme d'une couche continue.

3. Gant selon la revendication 1, dans lequel ladite partie de revêtement de côté de dos (5B) est agencée sous la forme d'une couche discontinue.

4. Gant selon la revendication 3, dans lequel ladite couche discontinue comprend un motif de points.

5. Gant selon la revendication 4, dans lequel des points (6) compris dans ledit motif de points sont répartis d'une manière uniforme sur la partie centrale de côté de dos (4B).

6. Gant selon l'une quelconque des revendications 1 à 5, comprenant un premier revêtement agencé au moins sur ladite partie de revêtement de côté de paume (5A), lequel premier revêtement présente une masse de revêtement totale se situant dans la plage de 5 à 20 g/gant de taille 10, la taille étant établie conformément à la norme EN 21420 ; et comprenant un second revêtement agencé au moins sur ladite partie de revêtement de côté de dos (5B), lequel second revêtement présente une masse de revêtement totale se situant dans la plage allant de 1 à 8 g/gant de taille 10.

7. Gant selon l'une quelconque des revendications 1 à 6, comprenant un premier revêtement agencé au moins sur ladite partie de revêtement de côté de paume (5A), lequel premier revêtement présente une masse de revêtement totale se situant dans la plage de 3,3 à 25 g ; et comprenant un second revêtement agencé au moins sur ladite partie de revêtement de côté de dos (5B), lequel second revêtement présente une masse de revêtement totale se situant dans la plage allant de 0,66 à 10 g.

8. Gant selon l'une quelconque des revendications 1 à 7, dans lequel le matériau résistant au feu comprend des polymères sélectionnés parmi le groupe constitué de silicium, de polychlorure de vinyle et de chloroprène, ou d'un mélange de ceux-ci.

9. Gant selon la revendication 8, dans lequel le matériau résistant au feu comprend de 10 à 90 % en poids de chloroprène, ou de 20 à 80 % en poids de chloroprène, ou de 30 à 70 % en poids de chloroprène, ou de 40 à 60 % en poids de chloroprène.

10. Gant selon l'une quelconque des revendications 1 à 9, dans lequel le revêtement résistant au feu comprend en outre un additif sélectionné parmi le groupe constitué : de pigments, d'agents de charge, de plastifiants, d'agents de surface, d'accélérateurs, d'agents de réticulation et d'agents de vulcanisation, ou de mélanges de ceux-ci.

11. Gant selon l'une quelconque des revendications 1 à 10, dans lequel la doublure de gant (2) est formée d'un matériau résistant au feu sélectionné parmi le groupe constitué : de paraaramide, de méta-aramide, de modacrylique, de coton, de laine, de polyamide et de polyester.

12. Procédé de fabrication d'un gant de protection contre les éclairs d'arc et résistant au feu (100, 200) comprenant les étapes consistant à :
- fournir une doublure de gant résistant au feu (2), laquelle doublure de gant (2) se compose d'un côté de paume (3) et d'un côté de dos (4), lequel côté de paume (3) comprend des parties pour doigts de côté de paume (3A), une partie centrale de côté de paume (3B) et une partie pour poignet de côté de paume (3C), lequel côté de dos (4) comprend des parties pour doigts de côté de dos (4A), une partie centrale de côté de dos (4B) et une partie pour poignet de côté de dos (4C) ;
- fournir un revêtement résistant au feu sur ladite doublure de gant (2) en :
fournissant une partie de revêtement de côté de dos (5B) présentant une surface d'au moins 4 cm² sur ladite partie centrale de côté de dos (4B) ; et
fournissant une partie de revêtement de côté de paume (5A) sur ledit côté de paume (3), où ladite partie de revêtement de côté de paume (5A) couvre au moins 90 % desdites parties pour doigts de côté de paume (3A) et au moins 90 % de ladite partie centrale de côté de paume (3B) ;
où une masse de revêtement moyenne de ladite partie de revêtement de côté de dos (5B) se situe dans la plage allant de 5 à 80 % d'une masse de revêtement moyenne de ladite partie de revêtement de côté de paume (5A) ; et
où ladite partie de revêtement de côté de dos (5B) est totalement ou partiellement composée d'un matériau résistant au feu différent par rapport à la partie de revêtement de côté de paume (5A).

13. Procédé selon la revendication 12, comprenant en outre les étapes consistant à :
- fournir au moins une composition de revêtement résistant au feu destinée à ladite partie centrale de côté de dos (4B),
- fournir au moins une composition de revêtement résistant au feu destinée audit côté de paume (3), et
- où ladite étape consistant à fournir un revêtement de côté de dos sur ladite partie centrale de côté de dos (4B) comprend en outre le fait de fournir au moins une couche de ladite au moins une composition de revêtement résistant au feu destinée à ladite partie centrale de côté de dos (4B) sur ladite partie centrale de côté de dos (4B),
- où ladite étape consistant à fournir un revêtement de côté de paume sur ledit côté de paume (3) comprend en outre le fait de fournir au moins une couche de ladite au moins une composition de revêtement résistant au feu destinée audit côté de paume (3) sur ledit côté de paume (3),
et où ladite composition de revêtement résistant au feu destinée audit côté de paume (3) et ladite composition de revêtement résistant au feu destinée audit côté de dos (4) sont différentes.

14. Procédé selon la revendication 13, dans lequel ladite étape consistant à fournir une partie de revêtement de côté de dos (5B) comprend en outre le fait de fournir une pluralité de couches de ladite composition de matériau résistant au feu les unes au-dessus des autres, et ladite étape consistant à fournir une partie de revêtement de côté de paume (5A) comprend le fait de fournir une pluralité de couches de ladite composition de revêtement de paume (5A) les unes au-dessus des autres, où
un nombre prédéterminé de ladite pluralité de couches de ladite partie de revêtement de côté de dos (5B) et un nombre prédéterminé de ladite pluralité de couches de ladite partie de revêtement de côté de paume (5A) sont fournis simultanément, par exemple au moyen d'un revêtement par immersion ou par pulvérisation ; et optionnellement le nombre total de couches de ladite partie de revêtement de côté de paume (5A) fournies sur ledit côté de paume (3) est supérieur au nombre total de couches de ladite partie de revêtement de côté de dos (5B) fournies sur la partie centrale de côté de dos (4B).

15. Procédé selon les revendications 12 à 14, dans lequel l'étape consistant à fournir ladite partie de revêtement de côté de dos (5B) et/ou ladite partie de revêtement de côté de paume (4B) est effectuée par un procédé comprenant une immersion, une pulvérisation, un brossage ou une sérigraphie, ou une combinaison de ceux-ci.

16. Procédé selon la revendication 15, dans lequel l'étape consistant à fournir ladite partie de revêtement de côté de dos (5B) comprend le fait de fournir un revêtement discontinu au moyen d'une pulvérisation ou d'une sérigraphie de ladite au moins une composition de revêtement résistant au feu destinée à ladite partie centrale de côté de dos (4B).
